

May 11, 1948.

B. M. PINELES

2,441,227

METHOD OF APPLYING TEMPORARY PROTECTIVE COATINGS

Filed April 27, 1944

2 Sheets-Sheet 1



Fig. 3

*Inventor*

Bernard M. Pineles

By his Attorney

*W.M.P.*

May 11, 1948.

B. M. PINELES

2,441,227

METHOD OF APPLYING TEMPORARY PROTECTIVE COATINGS

Filed April 27, 1944

2 Sheets-Sheet 2



*Inventor*  
Bernard M. Pineles  
*By his Attorney*  
*Manuel J. Delaney*

## UNITED STATES PATENT OFFICE

2,441,227

METHOD OF APPLYING TEMPORARY  
PROTECTIVE COATINGS

Bernard M. Pineles, Hamilton, Mass., assignor to  
United Shoe Machinery Corporation, Flemington, N. J., a corporation of New Jersey

Application April 27, 1944, Serial No. 533,015

3 Claims. (Cl. 117—6)

1

This invention relates to the method of applying by means of a spray a temporary protective coating of a film-forming colloid, which may be readily peeled or stripped off when desired, to an article having gaps or openings in its surface.

Many articles, to which films or coatings are to be applied, have gaps or openings in their surfaces. For example, the barrel of a machine gun is commonly surrounded by a hollow supporting jacket the wall of which has holes in it, and there are larger openings in the walls which enclose the firing mechanism. Examples of larger articles having openings which lead into their interiors are automobiles and airplanes. When such articles are to be coated it is desirable first to cover or bridge over all openings, except perhaps in certain cases very small ones, before applying to the article its temporary protective film or coating. It is possible, of course, to cover such openings by means of some extraneous material such as cloth, paper or adhesive tape, and then to spray on the solution of film-forming colloid.

According to the present invention the gaps or openings are bridged by means of a spray of a colloidal solution, the spray particles being in the form of long filaments which as they strike the article having openings to be bridged are comparatively dry; and then over these bridging coatings and over uncoated portions of the article there is applied, by means of a spray, the particles of which are smaller, probably globular or nearly so, and wetter than those of the bridging spray, a coating which amalgamates with and adheres firmly to the bridging coatings to form a tough, flexible, temporary protective coating which adheres lightly to the article and may be readily peeled or stripped off when desired. In practice a spray gun may be used to apply both the bridging coating and the superposed coating, the proportion of solid to liquid in the particles of spray material being varied to produce the comparatively dry filaments of the bridging coating or the wetter particles of the regular coating as may be desired.

Referring to the accompanying drawings,

Fig. 1 is a perspective of a machine gun in process of having an opening in its bottom covered by a bridging coating of filaments applied as a spray;

Fig. 2 is a perspective showing more particularly how the bridging coating is applied; and

Fig. 3 is a perspective of the same machine gun as is shown in Fig. 1 after all the openings have been covered by a bridging coating of comparatively dry filaments, and then a second super-

posed coating has been amalgamated with the lightly adherent bridging coating to form an integral coating covering the entire gun which may be readily stripped off when desired.

5 The machine gun 7 which is to be coated is supported upside down upon two crotched posts 9, 11 (both being shown in Fig. 3), the crotch of one post receiving an end of the barrel, and the crotch of the other post receiving a portion of a cylindrical member 13 at the rear of the gun. The machine gun, thus supported, may be rotated to expose all parts of its surface to the action of a spray which issues from a spray gun 17 held by the operator in one hand while with the other he rotates the machine gun as may be desired.

10 The spray gun is a commercial one, the emission of spray from the main nozzle being controlled by a trigger 19. The gun is provided with two valves 21, 23 which may be opened and closed by turning their knurled heads. The valve 23 controls the flow of spray material. The valve 21 does not control the flow of air through the main nozzle. When opened, it permits flow of extra air through two small auxiliary nozzles 24, 25 so as to provide more air and to flatten out the spray into the fan-shape shown. When the valve 21 is closed, the spray has the shape of a cone and the proportion of air to spray material is less than when the valve 21 is open. Air is supplied to the spray gun from an air compressor (not shown) through a tube 27, there being between the air compressor and the spray gun a valve (not shown) manipulation of which varies the pressure of the air. A second tube 29 leads from a source 15 of supply (not shown) under pressure of the solution of spray material to a small receptacle 31 which is fast to the spray gun, a valve (not shown) being provided for varying the pressure upon the spray material. When the valve 21 is closed and the spray, as has been stated, has the general form of a cone, the proportion of air to spray material passing through the main nozzle is so adjusted that the particles of spray are globular or nearly so and contain a comparatively 20 large amount of solvent, this spray being termed the regular wet spray as distinguished from the bridging spray, the particles of which are in the form of comparatively long, comparatively dry filaments. This latter spray may be produced by decreasing the proportion of spray material to air, for example by closing to a larger extent the valve 23. Preferably, however, the valve 23, which controls the flow of spray material, remains in its original position; and the valve 21 is opened to supply more air and to flatten out the spray into

the fan-shaped spray is shown, a comparatively thin flat fan-shaped spray being preferable in bridging certain openings in a manner which appears below.

The machine gun is shown as upside down with a generally rectangular opening in the bottom of the frame in process of being covered or bridged by a fan-shaped spray, the particles of which as has been stated are in the form of long, comparatively dry filaments. The operator preferably directs the spray as shown, at a small angle to the plane of the opening, and swings the spray gun somewhat back and forth in an arc, while maintaining substantially unchanged the angle referred to above. The filaments, which still contain a small amount of solvent when they strike the article, adhere lightly to the rim of the opening, and there results a bridging coating made up of filaments arranged at random. After all the openings, or at least all the large openings, have been covered by means of this bridging coating, the proportion of spray material to air is again adjusted to produce the spray referred to above as the regular wet spray, the particles of which are globular, or nearly so and contain a greater proportion of solvent to solid when they strike the machine gun than do the particles of the bridging spray; and this regular spray is used to apply a coating over the bridging coatings and over uncoated portions of the machine gun. The superposed coating adheres firmly to and amalgamates with the bridging coatings to form an integral coating which, like the bridging coatings, adheres lightly to the articles. The spray of filaments is somewhat drier than the regular spray and is referred to herein as a spray of long, comparatively dry filaments. This spray results in a lightly adherent coating; the following comparatively wet spray forms a coating which amalgamates with the bridging coating and adheres lightly to the article; and there results a single coating which may readily be peeled or stripped off.

With regard to the term "lightly adherent," the filaments adhere in a certain degree to the article and in a greater degree to each other so that a bridging coating of filaments more or less entangled and superposed at angles upon others beneath them is formed which remains in place while the somewhat wetter, more or less globular particles of the following spray are deposited upon it and form a coating which amalgamates with the bridging coating, said last-named particles being also deposited in the localities where there is no bridging coating, the amalgamated partly laminated coating being capable of being readily peeled or stripped off when desired. The above is true even though the article to be coated has upon it, as frequently happens when the article is a machine gun, a thin coating of light lubricating oil. At least it is certain that the bridging coating adheres lightly even under the above circumstances. As to the following coating in the case of an article such as a machine gun which has a light coating of oil, it may be that the lightly adherent quality of the enveloping coating is due in large measure to the shrinking which takes place when the solvent evaporates.

There is, of course, a limit to the size of an opening which may be bridged by the spray of filaments. Just what the limit is, is not known, but an opening, the smallest dimension of which is about 8", may readily be bridged. Only very

large articles or objects, such, for example, as airplane wheel housings have larger openings, and consequently in general no difficulty is encountered. Fig. 2, which is illustrative of how the bridging is done, shows a generally cylindrical ceramic vessel 31 with a circular opening in its top, said opening being considered for purposes of discussion to have a diameter of 8". The spray, as has been stated, is a thin, fan-shaped one. The filaments do not need, in this case, to be 8" long. They may be, say, 1"-3" long. As the spray strikes the locality of the rim of the receptacle nearest to the spray gun, some of these traveling filaments adhere to the rim and extend to some extent over the opening. Presently other filaments adhere to the free ends of the first filaments; and this process proceeds with following filaments until the filaments added one to another extend across the opening. The fan-shaped spray is held at a comparatively small angle to the plane of the opening, which in the figure is horizontal, and is swung back and forth in an arc while maintaining the angle substantially constant. There thus results a bridging coating made up of a network of filaments arranged at random, more or less tangled, and extending at different angles over others beneath them.

Assuming that the proportion of compressed air to spray material passing through the spray gun is such that the spray is what has been termed the regular spray and consists of globular or similarly shaped particles which, with the nozzle of the spray gun held at a convenient distance, say 4 or 5 inches, from the article, will produce what has been termed the wet coating, that is, one which will dry out to a tough, flexible, lightly adherent film, the procedure of applying a temporary protective coating to an article, such, for example, as a machine gun, which has openings in its surface, is as follows. The proportion of compressed air to spray material is increased, the valve 21 being preferably opened somewhat. There is thus produced a thin fan-shaped spray the particles of which are comparatively long, comparatively dry filaments. The spray gun is preferably held farther from the article, say 15", during the application of the bridging coatings. In the above specific example in which certain convenient distances have been given, the pressure upon the spray material may be 15 lbs. per square inch and that on the air 30 lbs. per square inch. After the openings have all been bridged by the use of this spray, the proportion of compressed air to spray material is decreased once more, for example, by closing the valve 21 to produce the regular spray of globular or similarly shaped particles which contain more solvent when they strike the articles than did the filaments of the bridging spray. The spraying is then continued with the spray gun held at, say, 4 or 5 inches from the article, to apply over the bridging coatings and over uncoated portions of the article what has been termed the regular wet coating, which amalgamates with the bridging coatings to produce with said bridging coatings a single coating which may be readily peeled or stripped off when desired. There has been described above a bridging coating and a superposed regular coating by the use of a single spray gun and the same spray material. It should be understood that the two spray coatings may, if desired, be of different materials provided that the spray materials are

compatible so that one coating will amalgamate with the other.

It is possible to use the regular spray to produce both the bridging coating and the superposed regular coating by first holding the spray gun at a considerable distance from the article sufficient to cause a large amount of evaporation of solvent to take place so that the particles of the spray are in the form of long, comparatively dry filaments when they strike the article, and then by holding the spray gun close to the article in applying the regular coating; but this procedure has the disadvantage that, when the spray gun is held at a sufficient distance from the article to produce suitable filaments, only a comparatively small number of spray particles strike the article at any given moment so that a considerable part of the spray material is wasted, and bridging the openings requires a much longer application of the spray. The other possibility, namely to make use only of the bridging spray and to hold the spray gun close to the article to produce the regular coating, involves an even more serious disadvantage in that the force of the compressed air, when the spray gun is held close to the article, is so great that holes are liable to be made in the bridging coating. Below are several examples of spray material.

#### Example I

|               | Parts by weight |
|---------------|-----------------|
| Vinylite VYNS | 15              |
| Acetone       | 85              |

Vinylite VYNS, a product of Carbide and Carbon Chemicals Corporation, of New York, is a copolymer of vinyl chloride and vinyl acetate containing about 88½% vinyl chloride.

#### Example II

|               | Parts by weight |
|---------------|-----------------|
| Vinylite VYNS | 10              |
| 3GH           | 5               |
| Acetone       | 85              |

3GH, a product of Carbide and Carbon Chemicals Corporation, of New York, is triethylene glycol di-2-ethyl butyrate and is a plasticizer specially designed for use with Vinylite resins.

#### Example III

|               | Parts by weight |
|---------------|-----------------|
| Vinylite XYSG | 10              |
| Methanol      | 90              |

#### Example IV

|               | Parts by weight |
|---------------|-----------------|
| Vinylite XYSG | 8               |
| 3GH           | 4               |
| Methanol      | 88              |

Vinylite XYSG, a product of Carbide and Carbon Chemicals Corporation, of New York, is an acetal which results from reacting polyvinyl alcohol with butyraldehyde.

#### Example V

|                                 | Parts by weight |
|---------------------------------|-----------------|
| Polymerized methyl methacrylate | 10              |
| Ethylene dichloride             | 90              |

#### Example VI

|                                 | Parts by weight |
|---------------------------------|-----------------|
| Polymerized methyl methacrylate | 10              |
| Dibutyl phthalate               | 5               |
| Ethylene dichloride             | 5               |

In the above examples the spray material con-

sists of a resin and a solvent with or without a plasticizer. It should be understood, however, that various other ingredients may be used if desired. For example, the spray material may have the following composition which, since it contains a corrosion inhibitor, forms part of the subject-matter of application Serial No. 736,514, filed March 22, 1947, which is a continuation in part of application Serial No. 533,014 filed April 27, 1944, now abandoned, in the names of John J. Brophy, Robert C. Putnam and myself.

#### Example VII

|                      | Parts by weight |
|----------------------|-----------------|
| 15 Vinylite VYNS     | 15              |
| 3GH                  | 4               |
| Oil 1255             | 4               |
| Glyceryl monolaurate | 4               |
| Acetone              | 85              |
| 20 Methyl Cellosolve | 10              |

Oil 1255, a non-corrosive, non-drying oil, is a product of the Standard Oil Company of New Jersey.

Having thus described my invention, what I claim as new and desire to secure by Letters Patent of the United States is:

1. The method of applying a temporary protective coating to an article having an opening in a wall thereof, said method comprising bridging the opening by causing a spray the particles of which are in the form of comparatively long, comparatively dry adhesive filament to travel across the opening in such manner that some of said filaments adhere to the rim of the opening and project over the opening and other filaments adhere to the projecting portions of said first-named filaments thereby progressively building up a bridging coating of a network of said filaments arranged at random, and then spraying the bridging coating and uncoated portions of the article with wetter and smaller adhesive spray particles to form with the bridging coating a tough, flexible, temporary protective coating which adheres lightly and may be readily stripped off when desired.

2. The method of applying a temporary protective coating to an article having an opening in a wall thereof, said method comprising providing a spray material in the form of a vinyl resin solution, causing a given amount of a gas under pressure to act upon a given amount of the spray material to produce a spray the particles of which comprise comparatively long, comparatively dry filaments, bridging the opening by directing said filament spray across the opening so that said filaments adhere to the rim of the opening and to one another to form a bridging coating, and thereafter decreasing the proportion of the gas to the spray material to produce a spray the particles of which are smaller and wetter than the spray of filaments and applying said spray over the bridging coating and over uncoated portions of the article to form a second coating which adheres firmly to the bridging coating and lightly to the article, whereby the two coatings become an integral one which may be readily stripped off when desired.

3. The method of applying a temporary protective coating to an article having an opening in a wall thereof, said method comprising bridging the opening by causing a thin generally fan-shaped spray the particles of which are in the form of comparatively long, comparatively dry filaments of film-forming colloidal material to

## REFERENCES CITED

The following references are of record in the file of this patent:

## UNITED STATES PATENTS

| Number    | Name    | Date          |
|-----------|---------|---------------|
| 1,954,219 | Moyses  | Apr. 10, 1934 |
| 2,314,329 | Ericson | Mar. 23, 1943 |

## FOREIGN PATENTS

| Number  | Country       | Date         |
|---------|---------------|--------------|
| 551,619 | Great Britain | Mar. 3, 1943 |

BERNARD M. PINELES.

7  
travel over the opening in such manner as to build up a bridging coating, and then causing a generally cone-shaped spray the particles of which are smaller and wetter than the filaments to travel over the bridging coating and over uncoated portions of the article to form with the bridging coating a tough, flexible temporary protective coating which adheres lightly and may be readily stripped off when desired.

5  
10